

May 12, 1942.

G. J. SNYDER

**2,282,432**

**BUILDING COVERING MEMBER**

Filed April 22, 1939

FIG. 1.



FIG. 2.



FIG. 3



FIG. 5



FIG. 4.



GILBERT J. SNYDER  
Attach & Knoblock  
INVENTOR.  
ATTORNEY'S

## UNITED STATES PATENT OFFICE

2,282,432

## BUILDING COVERING MEMBER

Gilbert J. Snyder, South Bend, Ind., assignor to  
 Mastic Asphalt Corporation, South Bend, Ind.,  
 a corporation of Indiana

Application April 22, 1939, Serial No. 269,542  
 In Canada November 14, 1938

2 Claims. (Cl. 117—56)

This invention relates to improvements in building covering members, and particularly to material of this character comprising a panel of rigid composition board of compressed cellulose fibers coated with waterproof material and surfaced to simulate the appearance and texture of a section of a masonry wall. This application is a continuation in part of my application, Ser. No. 174,597, upon which Letters Patent No. 2,164,725 issued July 4, 1939.

Exterior building covering members formed of composition board and coated with waterproof material such as asphalt have a serious objection in that they have a tendency to peel, especially when struck or pulled at an edge. This is a definite peeling or delamination of the board itself, as distinguished from a separation of the coating from the board. Asphalt has a stronger adhesion with the board than the adhesion between fibrous constituents of the board, hence the delamination above mentioned. Also, the asphalt is flexible, and this quality enhances and increases the likelihood of delamination, especially when once started at an edge of the panel, as when the same has been struck.

It is, therefore, the primary object of this invention to provide a building member formed of composition board and coated with asphalt or the like, wherein the tendency of the board to peel beneath the coating when struck at its edge is substantially completely eliminated.

A further object is to provide a member of his character wherein the outer surfaces of the board are surface saturated to bind the fibers hereof and rigidify and strengthen the board.

A further object is to provide a composition board product of this character of increased strength and rigidity and with insulating properties substantially unimpaired.

Other objects will be apparent from the description and appended claims.

In the drawing:

Fig. 1 is a face view of my improved building member.

Fig. 2 is a fragmentary enlarged sectional view taken on line A—A of Fig. 1.

Fig. 3 is a fragmentary enlarged sectional view similar to Fig. 2 and illustrating the manner of tailing the member.

Fig. 4 is a fragmentary enlarged sectional view of the saturated composition board base with a reformed nail hole.

Fig. 5 is an enlarged fragmentary sectional view similar to Fig. 2 illustrating a modified construction of building member.

Referring to the drawing, the numeral 10 designates a building covering member having marginal ship lap flanges 11 and a coated contoured face provided with longitudinal and transverse 5 narrow elongated depressions 12 arranged to simulate mortar joints and separating surface areas simulating masonry members such as bricks 13.

The member is preferably formed on a base 10 best illustrated in Fig. 4, which constitutes a rigid panel 14 of composition board of compressed cellulose fibers, such as "Celotex" and the like. A plurality of spaced narrow holes 15 are formed in and extend through the board 14 in predetermined relation and arrangement. The entire surface portion of the board is saturated to a comparatively shallow depth with waterproof material such as asphalt 16, said saturant also saturating the board at 17 at the walls of each hole 15. Composition board is of compressed fibrous character whereby it has substantially greater porosity at its edges than at its faces, whereby the transversely extending saturated portions, as at 17 around holes 15 are of greater depth than 20 face portions 16. This effectively reinforces the board at its weakest points, as around ship lap flanges 11, and also serves to form a binder for the laminations of the composition board around each nail hole. The saturant preferably penetrates to only a shallow depth sufficient to provide the improved structural and waterproof characteristics without impairing the insulating properties of the composition board to any material extent.

25 The preformed composition board above described may be treated and finished to provide any of several well known types of finished product. One such type is illustrated in Fig. 2 wherein a continuous surface layer or coating 18 of asphalt or like waterproof material is applied to one face of the preformed panel; and colored granular material or grit 19 is applied to coating 18. This coating is suitably pressed to provide the depressions 12 therein, and thus achieve 30 the masonry simulation. The depressions are preferably located to coincide with the various holes 15 in the board 14, and the formation thereof tends to force the coating material into the upper ends of holes 15 to a substantial extent.

35 At 20, as illustrated in Fig. 2. At the same time the depressions 12 are formed, as by suitable dies, indentations 21 may be formed in coating 18 in registering relation to the holes 15. In applying this type of member to a building, the panel 40 is applied flat against a building 22 as against

45

50

55

studding, sheathing, siding or the like, and nails 23 are driven therethrough at holes 15 and into the building. The nail heads seat in depressions 12, and are completely protected and concealed by waterproofing material at 24.

Another embodiment of the invention is illustrated in Fig. 5, wherein the preformed partially saturated composition board 14 is likewise coated with a comparatively thin continuous layer 18 of adhesive waterproof material sealing one end of holes 15 at 20 and indented at 21 in registration with each hole 15. In this construction, however, the coating 18 serves to cause thin slab units 25 of brick, stone, asbestos composition or the like to adhere to the base in spaced patterned relation. Nails are adapted to be driven through holes 15 in the spaces between slabs 25 to secure the unit to a building as heretofore described, the space then being filled with mortar or like material (not shown) which conceals the 20 nails and completes the surface.

It will be seen that, with both above described types of construction, the nail pierces the portion 20 of coating 18 in holes 15 and passes through said holes in the member without exposing or contacting an unsaturated portion of the board. The increased depth of penetration of the saturant at areas 17 around holes 15 insures against such contact of the nails with unsaturated portions of the board even when the 30 nail is driven at an angle to hole 15; and also serves as a reinforcement to prevent damage to the board if a nail is driven so deeply as to lodge its head below the upper surface of the base. The nails employed are preferably of slightly greater thickness than the transverse dimension of holes 15 so as to insure a tight fit of the nails with the board, and the saturant 17 around the holes 15 insures a binding or adhesive contact as well as a frictional fit between the nail and board. In addition, the saturation of portion 17 around the nail increases the strength of the board where it is nailed and insures solid effective anchoring of the unit to the building when nailed. In this way fewer nails are required to secure my improved member solidly to a building than are required to secure a conventional unsaturated member of the same character and size. Furthermore, in the event fewer nails are employed than provided for, the unused nail 50 holes 15 remain permanently and effectively sealed in weatherproof manner by portions 20 of coating 18 at the outer ends of said holes, so that the presence of such holes will not detract from the weatherproof character of the building member. The indentations 21 which indicate the locations of such unused nail holes are small and inconspicuous, and these factors coupled with the location of the indentations in depressions 12 does not detract from the general appearance of the members and renders the presence of unused nail holes therein unnoticeable when said members are applied on a building. It will, of course, be understood that one of the prime advantages of this construction is the retention of the insulating value of the base by retaining the major portion thereof unsaturated, while at the same time preventing moisture from entering the unsaturated interior of the body by way of the nail holes. In this connection, it 70 will be noted that the construction is particularly effective with the type of construction shown in Fig. 5 where the slabs 25 render each building unit quite heavy and nailing of the unit

5 tends to deform the board around the hole and to enlarge the hole by reason of said weight, all of which is avoided by the saturation reinforcement of the base as described. Additionally, the Fig. 5 type of construction contemplates the use of regular mortar between slabs without coating the nail heads, the moisture from the mortar thus being directly accessible at the points of nailing, so that any looseness between nail and member in conventional construction permits the moisture to enter the same, whereas all such dangers are eliminated by the instant construction.

15 For the purpose of stabilizing the product, the saturating agent employed is preferably an asphalt having a comparatively high melt point and substantially free from volatile solvents, and the coating 18 is formed of like material. In this way all possibility of chemical action between the coating and saturant, such as permeation of coating 18 by solvents which dilute the body thereof or impair the adhesive qualities thereof, is avoided.

25 Attention is also directed to the fact that, with respect to the feature of the tight sealed fit between the board and nails and the waterproof character of the board around the nail, it is possible to avoid or eliminate use of coating 24 over the nail head in the Fig. 3 type of construction, by using rust proof nails of the same color at their heads as the color or coating 18, usually black. In other words, the construction is so sealed around the nail that protection of the board by such coating is unnecessary, and the 35 color problem for concealment of the nail is all that must be considered.

40 The surface saturation of the composition board binds together the surface fibers of the board and rigidifies the same. The saturation underlying the coated face cooperates with the 45 coating to rigidify the same; while that at the edges resists separation of the fibers and damage to the board at its edges. Both thus serve positively to minimize possibility of delamination of the board by peeling of the coating therefrom.

I claim:

1. A building covering member comprising a rigid composition board formed of compacted fibrous material which is subject to peeling when coated with flexible plastic material, waterproof material impregnating said board to a shallow depth at all surfaces thereof whereby the fibrous material at all edges of said board is firmly bound together, and a coating of bituminous material covering one surface of said board, the depth of impregnation of the board portion underlying said coating being sufficient to substantially increase the rigidity of said portion and the coating adhering thereto and thereby resist peeling of said board, the major portion of the board being unsaturated to substantially retain the insulation properties of the board.

2. A building covering member comprising a rigid composition board formed of compacted fibrous material which is subject to peeling when 65 coated with flexible plastic material, a coating of flexible plastic waterproof material covering one surface of said board, and adhesive material binding the fibrous material of the board at all edges thereof to resist peeling of said board without substantially impairing the insulation properties of the board.

GILBERT J. SNYDER.